

# United States Patent Office

2,866,740

Patented Dec. 30, 1958

1  
2,866,740

## ELECTRODEPOSITION OF RHODIUM

Frank Herbert Reid, Hounslow, England, assignor to The International Nickel Company, Inc., New York, N. Y., a corporation of Delaware

No Drawing. Application May 2, 1957  
Serial No. 656,499

Claims priority, application Great Britain May 10, 1956

9 Claims. (Cl. 204—47)

The present invention relates to the electro-deposition of rhodium and, more particularly, to the deposition of crack-free rhodium electrodeposits.

Electrodeposits of rhodium both for decorative and industrial purposes are well known. The so-called decorative deposits are used, for example, in the protection of silverware and base metals and also in scientific apparatus. Industrial deposits, which are thicker than decorative deposits and are resistant to corrosion and to mechanical wear, are used, inter alia, as the surfaces of sliding electrical contacts. The thickness of a decorative deposit is generally between 0.000005 and 0.00005 inch, and that of an industrial deposit is generally between 0.0001 and 0.002 inch or greater. The electrolytes commonly used are solutions of rhodium sulphate containing various concentrations of sulphuric acid; but other acid solutions, for example, of rhodium phosphate or fluoborate, can be used. A substantially unidirectional electric current is passed through these baths and rhodium is deposited at the cathode.

Rhodium deposits as produced from the prior art baths show a pronounced internal tensile stress, which is dependent to some extent on the deposition conditions, but is generally of a high order, e. g., 50 to 100 tons/in.<sup>2</sup>. In deposits thicker than about 0.0001 inch, the stress often leads to cracking of the rhodium deposit in the "as plated" condition. Cracks formed in this way may be referred to as primary cracks and usually extend right through the deposit to the basis metal. They may be detected by the so-called electrographic method, in which the basis metal, which is exposed by the cracking, is made to produce a pattern on a suitable test paper. Cracks are of course undesirable, particularly when the object upon which rhodium is deposited is exposed to a corrosive environment and my object is to reduce or eliminate this cracking tendency.

Although many attempts were made to overcome the foregoing difficulties and other disadvantages, none, as far as I am aware, was entirely successful when carried into practice commercially on an industrial scale.

It has now been discovered that by the use of novel rhodium electroplating baths, substantially crack-free electrodeposits may be produced under normal commercial electroplating conditions.

It is an object of the present invention to provide a novel electrochemical plating bath which enables one to reduce or substantially eliminate cracks in rhodium electrodeposits.

Other objects and advantages will become apparent from the following description.

Generally speaking, the present invention contemplates the production of electrodeposits of rhodium through the use of an aqueous, acidic electrodeposition bath which contains a soluble rhodium salt and at least sufficient free mineral acid to prevent hydrolysis of the selected rhodium salt and selenium in an amount equiva-

lent to about 0.05 gram per liter (g. p. l.) to about 25 g. p. l. of selenic acid. It is preferred to add at least about 0.05 g. p. l. of selenic acid and/or of one or more salts of said acid to the rhodium plating bath in order to provide an amount of selenate ion therein which is effective in reducing the primary cracking tendency of the deposit. The soluble rhodium salt sufficient to provide from about 5 to 20 grams per liter of dissolved rhodium, for example, about 10 g. p. l., may be selected from the group consisting of rhodium sulphate, rhodium phosphate and rhodium fluoborate. The free acid may be selected from the group consisting of sulphuric acid, phosphoric acid and fluoboric acid and may be employed in amounts at least up to about 100 milliliters per liter (m. p. l.). The necessary concentration of selenic acid is supplied either by the addition of the acid itself or by the addition of a salt which upon hydrolysis in the presence of a mineral acid will produce a satisfactory effective quantity of selenic acid. Of course, when adding the hydrolyzable salt, it is preferred that the reaction products of the hydrolysis reaction will not interfere with the electrodeposition. Accordingly, it is preferred to use a sodium or other alkali metal salt of selenic acid when a salt addition is indicated.

25 In carrying the invention into practice, it is preferred to provide a range between a minimum of at least 0.05 g. p. l. to a maximum of about 1 g. p. l. (or even a maximum of about 8 g. p. l.) of selenic acid in the aqueous acidic rhodium electroplating bath. I prefer to add free selenic acid. Although any addition of selenic acid will reduce the cracking to some extent, I prefer always to add at least 0.05 g. p. l. The amount necessary to ensure practical freedom from cracking under all conditions of deposition is about 0.4 g. p. l. in an electrolyte low in free mineral acid, e. g., sulphuric acid, and rather less in an electrolyte with a higher concentration of free mineral acid, e. g., sulphuric acid. No advantage is gained by adding more than 8 grams of selenic acid per liter. Rhodium sulphate is the preferred source of dissolved rhodium and a preferred electrolyte according to the invention may thus have the following composition:

|                       |                         |
|-----------------------|-------------------------|
| Rhodium (as sulphate) | 5 to 20 gms./liter.     |
| Free sulphuric acid   | Up to 100 mls./liter.   |
| Selenic acid          | 0.05 to 0.8 gms./liter. |

30 The temperature of operation and the current density are not affected by the addition of selenic acid. The temperature may be from about 20° C. to about 70° C., preferably above 50° C., and the current density from about 0.5 to about 2 amperes per square decimeter (amps./dm.<sup>2</sup>). Especially advantageous results are obtained when the current density is about 1 amp./dm.<sup>2</sup>. Rhodium sulphate electrolytes are commonly made by dilution of concentrated solutions, themselves made by dissolving rhodium hydroxide in sulphuric acid. As a general rule, therefore, the electrolyte contains a small amount of free sulphuric acid. Further sulphuric acid is often added to increase the content of free sulphuric acid.

35 While it is to be observed that the present invention contemplates the minimization of primary cracking tendency in rhodium electrodeposits produced over a broad range of operating conditions, certain relationships between operating conditions and bath composition should be maintained in order to assure the best results. For example, if the temperature is maintained on the low side of the aforementioned range, the concentration of free mineral acid should be increased. From the standpoint of smoothness of deposit, an operating temperature of about 50° C. has been found to be most effective. Using the same criterion, a current density of about 1

amp./dm.<sup>2</sup> has been found to provide optimum results. Again it is to be noted that as the concentration of selenic acid is increased, the hardness of the rhodium deposit is decreased due to an increase in selenium content in the deposit. Thus, one should introduce a maximum of about 1 g. p. l. of selenic acid into the bath where hardness of the deposit is an important characteristic of the deposit. As was indicated hereinbefore, to achieve optimum minimization of primary cracking tendency, the amount of selenic acid added to the electrolyte should be increased as the amount of free mineral acid is decreased. As a general rule, it is preferred to add a minimum of 0.4 g. p. l. of selenic acid to the electrolyte regardless of the free mineral acid concentration.

It is to be observed that the present invention contemplates a more advantageous rhodium electrodeposition bath which contains ingredients in the following tabulated ranges of concentration in units of g. p. l.

TABLE I

| Ingredients               | Broad               | Desired    |
|---------------------------|---------------------|------------|
| Rhodium (as soluble salt) | 5-20                | about 10.  |
| Free Mineral Acid         | 12-100 <sup>1</sup> | >about 20. |
| Selenic Acid              | 0.05-25             | about 1.   |
| Water                     | Balance             | Balance.   |

<sup>1</sup> Milliliters per liter

Likewise, the operating conditions are tabulated in Table II:

TABLE II

| Conditions                             | Broad | Desired |
|----------------------------------------|-------|---------|
| Temperature, °C.                       | 20-70 | 50      |
| Current Density, amp./dm. <sup>2</sup> | 0.5-2 | 1       |

It is to be observed that while the specification has disclosed that the electrodeposits produced from the aforementioned baths of the present invention are of metallic rhodium, they contain small amounts of selenium, the amount thereof depending to a certain extent on the concentration of selenic acid used in the bath. For purposes of this specification, it is intended that the terms "rhodium" or "electrodeposited rhodium" when used in reference to the electrodeposits include these small amounts of selenium. In view of the inclusion or codeposition of selenium with rhodium, it should be noted that when the baths disclosed herein are replenished, not only rhodium must be added thereto but also suitable additions of selenic acid should be made.

For the purpose of giving those skilled in the art a better understanding of the invention, the following illustrative examples are given:

#### Example I

A rhodium plating electrolyte was made by dissolving rhodium hydroxide in sulphuric acid and diluting the resulting solution to a concentration of 10 gms./liter of rhodium as sulphate. No further additions of sulphuric acid were made. A deposit 0.0007 inch thick produced from this electrolyte at a temperature of 45° C. with a current density of 2 amp./dm.<sup>2</sup> showed severe cracking.

After adding selenic acid to the electrolyte to give a concentration of 0.4 gms./liter, an uncracked deposit 0.001 inch thick was obtained under the same operating conditions.

#### Example II

##### Electrolyte composition:

Rhodium (as sulphate) \_\_\_\_\_ gms./liter 10  
Added sulphuric acid \_\_\_\_\_ mls./liter 70

A deposit 0.0007 inch thick obtained from this electrolyte at a temperature of 45° C. with a current density

of 2 amp./dm.<sup>2</sup> showed moderate cracking. After addition of selenic acid to give a concentration of 0.4 gm./liter, an uncracked deposit 0.0012 inch thick was obtained.

#### Example III

U-shaped specimens of copper rod were plated in an electrolyte of the composition given in Example II both before and after the addition of selenic acid to give a concentration of 0.4 gm./liter. The thickness of rhodium in each case was 0.0005 inch. The specimens were then immersed in concentrated nitric acid. After 25 minutes the specimen plated before the addition of selenic acid had completely dissolved, whereas the other specimen was unaffected.

#### Example IV

Flat copper specimens were plated on one side only with rhodium deposits 0.0005 inch thick from the electrolytes of Example III. The copper was then dissolved away by treatment with nitric acid. The deposit from the electrolyte that was free from selenic acid disintegrated into numerous fine flakes because of cracks in it, but the deposit from the treated electrolyte remained as a coherent foil.

The present invention is particularly applicable to the electrodeposition of rhodium on any metal which is compatible with the acid electrolytes. These metals include nickel, nickel-silver, silver, gold, platinum, palladium, copper and brass.

It is to be observed that the present invention provides a process for the production of deposits of rhodium having reduced cracking tendencies from an acid electrolyte and also provides a novel acidic electrolyte for the production of such rhodium electrodeposits.

Although the present invention has been described in conjunction with preferred embodiments, it is to be understood that modifications and variations may be resorted to without departing from the spirit and scope of the invention, as those skilled in the art will readily understand. Such modifications and variations are considered to be within the purview and scope of the invention and appended claims.

I claim:

1. An electrolyte for producing substantially crack-free rhodium electrodeposits comprising an aqueous acidic bath containing dissolved rhodium derived from at least one compound from the group consisting of rhodium sulphate, rhodium phosphate and rhodium fluoroborate in an amount to provide from about 5 to about 20 grams per liter of rhodium, free acid in an amount sufficient to prevent hydrolysis and a compound from the group consisting of selenic acid and alkali metal salts thereof in an amount equivalent to about 0.05 to about 25 grams per liter of selenic acid.

2. An electrolyte for the production of substantially crack-free rhodium electrodeposits comprising an aqueous acid bath containing dissolved rhodium derived from at least one compound from the group consisting of rhodium sulphate, rhodium phosphate and rhodium fluoroborate in an amount to provide from about 5 to about 20 grams per liter of dissolved rhodium, an acid from the group consisting of sulphuric acid, phosphoric acid and fluoroboric acid in an amount sufficient to prevent hydrolysis of the rhodium compound but not substantially exceeding about 100 milliliters per liter of electrolyte and a compound from the group consisting of selenic acid and alkali metal salts thereof in an amount equivalent to about 0.05 to about 8 grams per liter of selenic acid.

3. A rhodium plating electrolyte for producing hard, substantially crack-free rhodium electrodeposits comprising an aqueous acidic bath containing dissolved rhodium derived from at least one compound from the group consisting of rhodium sulphate, rhodium phosphate and rhodium fluoroborate in an amount to provide about 10 grams per liter of dissolved rhodium, from about 12 to

about 100 milliliters per liter of sulphuric acid and about 0.05 to about 1 gram per liter of selenic acid.

4. The process for producing substantially crack-free electrodeposits of rhodium which comprises establishing an aqueous acidic electrolyte containing about 5 to about 20 grams per liter of rhodium, from about 12 to about 100 milliliters per liter of free acid selected from the group consisting of sulphuric acid, phosphoric acid and fluoboric acid, at least about 0.05 up to about 1 gram per liter of selenic acid, and electrolyzing said bath at a current density of about 0.5 to about 2 amperes per square decimeter and a temperature of about 50° C. to produce a rhodium electrodedeposit characterized by being substantially free from cracking.

5. The process for producing substantially crack-free electrodeposits of rhodium which comprises establishing an aqueous acidic electrolyte containing about 5 to about 20 grams per liter of rhodium, from about 12 to about 100 milliliters per liter of free sulphuric acid and about 0.4 gram per liter of selenic acid, and electrolyzing said bath at a current density of about 1 ampere per square decimeter and a temperature of about 50° C. to produce a rhodium electrodedeposit characterized by being substantially free from cracking.

6. A rhodium plating bath for producing substantially crack-free rhodium electrodeposits comprising an aqueous acidic electrolyte containing in solution about 5 to about 20 grams per liter of rhodium, free acid in an amount sufficient to prevent hydrolysis of said rhodium and selenate ion in an amount equivalent to a concentration of at least about 0.05 up to about 25 grams per liter of selenic acid.

7. A rhodium plating bath for producing substantially crack-free rhodium electrodeposits comprising an aqueous acidic electrolyte containing in solution rhodium derived from at least one compound from the group consisting of rhodium sulphate, rhodium phosphate and rhodium fluoborate in an amount to provide from about 5 to about 20 grams per liter of dissolved rhodium, from about 12 to about 100 milliliters per liter of free acid from the group consisting of sulphuric acid, phosphoric acid and fluoboric acid and selenate ion in an amount equivalent to about 0.05 to about 1 gram per liter of selenic acid.

8. The process for producing substantially crack-free electrodeposits of rhodium which comprises establishing an aqueous acidic electrolyte containing in solution about 5 to about 20 grams per liter of rhodium, free acid in an amount sufficient to prevent hydrolysis of said rhodium and selenate ion in an amount equivalent to a concentration of at least about 0.05 up to about 25 grams per liter of selenic acid and electrolyzing said bath at a current density of about 0.5 to about 2 amperes per square decimeter and a temperature of about 20° C. to about 70° C. to produce a rhodium electrodedeposit characterized by being substantially free from cracking.

9. The process for producing substantially crack-free electrodeposits of rhodium which comprises establishing an aqueous acidic electrolyte containing in solution about 5 to about 20 grams per liter of rhodium, free acid selected from the group consisting of sulphuric acid, phosphoric acid and fluoboric acid in an amount sufficient to prevent hydrolysis of said rhodium but not substantially exceeding about 100 milliliters per liter of electrolyte and a compound from the group consisting of selenic acid and alkali metal salts thereof in an amount equivalent to a concentration of at least about 0.05 up to about 8 grams per liter of selenic acid and electrolyzing said bath at a current density of about 0.5 to about 2 amperes per square decimeter and a temperature of about 20° C. to about 70° C. to produce a rhodium electrodedeposit characterized by being substantially free from cracking.

30

References Cited in the file of this patent

UNITED STATES PATENTS

|           |              |                |
|-----------|--------------|----------------|
| 2,384,501 | Streicher    | Sept. 11, 1945 |
| 2,461,933 | Smith et al. | Feb. 15, 1949  |
| 2,577,365 | Reid         | Dec. 4, 1951   |

FOREIGN PATENTS

|         |               |              |
|---------|---------------|--------------|
| 440,938 | Great Britain | Jan. 8, 1936 |
|---------|---------------|--------------|

OTHER REFERENCES

40 Weisner et al.: "Plating," vol. 43 (March 1956), pp. 347-355.